

## UNITED STATES PATENT OFFICE.

LEO SMITH, OF MANCHESTER, ENGLAND, ASSIGNOR TO BRITISH DYESTUFFS CORPORATION LIMITED, OF MANCHESTER, ENGLAND.

DIECHARGE EFFECTS ON MATERIALS CONSISTING WHOLLY OR IN PART OF ACETYL CELLULOSE.

No Drawing. Application filed September 23, 1926, Serial No. 137,389, and in Great Britain November 25, 1925.

It is well known that the reduction discharge processes based on sodium sulphoxylate in general use for the production of discharge effects on cotton, silk and woolen materials are not effective when applied to acetyl cellulose. For this reason a large and important range of designs cannot be produced at the present time on materials consisting either wholly or in part of acetyl cellulose.

A typical reduction discharge is that in which use is made of products sold under the various trade names and depending upon their sodium formaldehyde-sulphoxylate content for their reducing properties.

Such typical reduction discharge printing pastes containing sodium sulphoxylate, will give a perfectly white discharge when applied by the usual methods to cotton, or other cellulose materials, which have for instance been dyed with chlorazol fast orange G, (dianil brown 3GO-Color Index No. 273) but it has very little effect when applied by the same methods to acetyl cellulose dyed with the same dyestuff.

I have found that the addition of sulphocyanides to the reduction discharge printing paste containing sodium sulphoxylate brings about complete reduction of all colours which are dischargeable when dyed on the usual textile materials by the use of the aforesaid discharge printing paste, but which hitherto have not been found dischargeable by the same process when dyed on acetyl cellulose materials. The sulphocyanides of calcium, barium and ammonium are typical but I do not limit myself to these.

Further, azo dyestuffs specially designed for the dyeing of acetyl cellulose materials such as the Ionamine series, manufactured by British Dyestuffs Corporation Limited. The dyestuffs formed by coupling dimethyl or diethyl-aniline with diazotised 5-nitro-o-anisidine or with diazotised 2:4-dinitroaniline (known as S. R. A. Reds, 1, 3 and 5), or by coupling diphenylamine with (S. R. A. Orange 1), or other S. R. A. dyestuffs manufactured by the British Celanese Limited, which also are not satisfactorily discharged by the usual discharge printing pastes containing sodium sulphoxylate, are found to give perfect whites if sulphocyanides are added.

Dependent for its success upon the attainment of a satisfactory white discharge of the ground colour, the so-called coloured discharge process, in which a suitable basic colour is added to the discharge printing paste containing sodium sulphoxylate, is correspondingly improved by the addition of sulphocyanides to the coloured discharge printing pastes.

*Example 1.*

A fabric consisting of cotton and acetyl cellulose is dyed in the customary manner with chlorazol fast Orange G. and is afterwards printed with a discharge printing colour made up as follows:—

15 grammes sodium formaldehyde-sulphoxylate are dissolved in 70 grammes of gum tragacanth solution—containing 30 grammes of gum tragacanth in one litre—and when in complete solution, 10 grammes calcium sulphocyanide solution 88° Tw. 75 (containing approximately 762 grammes calcium sulphocyanide in one litre) are added. After the fabric has been printed, it is dried and then aged for 3 to 5 minutes in any ordinary type of rapid ageing 80 machine at 100° C. It is then washed in water at 60° C. for three minutes and dried.

*Example 2.*

Material consisting of acetyl cellulose is dyed in the usual manner with the formaldehyde bisulphite compound of 3-nitro-4'-aminoazobenzene, obtained by coupling m-nitrodiazobenzene with aniline, and treating the product with formaldehyde and sodium bisulphite solution and is afterwards diazotised and developed with beta-naphthol in the customary way. It is then printed and after-treated as described in Example 1.

*Example 3.*

Material consisting of acetyl cellulose is dyed in the usual way with S. R. A. Orange 1 (British Celanese Ltd.) which is 4-nitrobenzeneazodiphenylamine and then it is printed and after-treated as described in Example 1.

*Example 4.*

Material consisting of acetyl cellulose is dyed, printed and after-treated as described

2  
in Example 1, except that Thionine Blue GO (color Index No. 926) is added to the discharge printing colour.

What I claim and desire to secure by Letters Patent is:—

1. The process of making a preparation for the production of discharge effects on acetyl cellulose materials which comprises the addition of sulphocyanides to the usual sodium formaldehyde-sulphoxylate discharge printing pastes.

2. As a new article of manufacture, a preparation for the production of discharge effects on materials containing acetyl cellulose comprising the usual sodium formaldehyde-sulphoxylate discharge printing paste and also comprising a sulphocyanide.

3. As a new article of manufacture, a preparation for the production of discharge effects on materials containing acetyl cellulose comprising the usual sodium formaldehyde-sulphoxylate discharge printing paste

and also comprising a sulphocyanide of an alkaline earth metal.

4. As a new article of manufacture, a preparation for the production of discharge effects on materials containing acetyl cellulose comprising the usual sodium formaldehyde-sulphoxylate discharge printing paste and also comprising calcium sulphocyanide. 30

5. As a new article of manufacture, a preparation for the production of discharge effects on materials containing acetyl cellulose comprising sodium formaldehyde-sulphoxylate, gum tragacanth, calcium sulphocyanide and water substantially in the proportions of 15 parts of sodium formaldehyde-sulphoxylate, 2.1 parts of gum tragacanth, 11 parts of calcium sulphocyanide and 71.4 parts of water, the parts being by 40 weight.

In testimony whereof I have signed my name to this specification.

LEO SMITH.